

## 1

3,322,657

**ELECTRODEPOSITION OF BRIGHT COPPER**  
 Karl-Wilhelm Sassenroth, Dusseldorf, Georg Jansen,  
 Neuss (Rhine), and Robert Brugger, Bernhausen, near  
 Stuttgart, Germany, assignors to Langbein-Pfanhauser  
 Werke A.G., Neuss (Rhine), Germany  
 No Drawing. Filed May 11, 1964, Ser. No. 366,628  
 6 Claims. (Cl. 204—52)

This invention relates to the electrodeposition of copper from acid electrolytes, and more particularly to the deposition of bright smooth copper coatings free from pores from acid electrolytes.

Acid copper plating solutions normally yield dull or semi-lustrous deposits with relatively poor throwing power. Known addition agents are capable of improving brightness, leveling ability, freedom from pores, or ductility of the deposit, but a combination of these properties is not readily obtained by known addition agents, and it is difficult to maintain satisfactory performance of a copper plating bath with respect to all the factors enumerated. It is generally necessary to provide an acid copper plating solution with at least one addition agent for each of the properties to be influenced. The multiple addition agents are lost from the plating bath by drag-out or decomposition at different rates, and their presence is not usually capable of being determined by simple chemical or physical analysis.

An object of the invention is the provision of an acid copper electroplating bath containing a source of copper ions and a source of hydrogen ions as is conventional, and producing copper electrodeposits which combine the afore-mentioned desirable properties to a very high extent with the use of a very small number of addition agents, preferably no more than two.

Another object is the provision of a new combination of addition agents for copper plating solutions which has good levelling effects, prevents the formation of pores due to hydrogen bubbles, and does not embrittle the copper deposits formed.

Yet another object is the provision of brighteners which are insensitive to relatively high concentrations of impurities in the plating bath, and thus permit operation over extended periods without requiring purification of the electrolyte.

We have found that the above objects are achieved by a combination of addition agents one of which is an N-tetrahydropyran-2 substituted amide of a carboxylic or thiocarboxylic acid. A wide variety of such amides may be used in acid copper plating solutions in amounts as low as 0.2 millimole per liter. The porosity and ductility of the deposits is not unfavorably influenced when the concentration of such primary addition agents is raised to their limit of solubility or 0.01 mole per liter whichever is lower.

The primary addition agents of the invention are of the formula



wherein X is either oxygen or sulfur, R is hydrogen or the radical of propane- $\omega$ -sulfonic acid, and R' may be any one of a large number of radicals to complete the struc-

## 2

ture of an N-tetrahydropyran-2 substituted carboxylic or thiocarboxylic acid amide, and more specifically that of an N-tetrahydropyran-2-substituted urea or thiourea, as will hereinafter become apparent.

The primary addition agents of the invention in which R is hydrogen are prepared in yields of 20 to 70 percent from 2,3-dihydropyran and amides corresponding to the brightening compounds to be produced in the presence of catalytic amounts of hydrogen chloride according to a method presented to the 139th meeting of the American Chemical Society, 1961, by A. I. Spezzale, K. W. Ratts, and G. I. Marco (J. Org. Chem., 26, 4311-14, 1961; C. A., 56, 14218, 1962; Angew. Chem., 1961 (73), 497). The compounds prepared in this manner readily react with propane sultone to form the corresponding N-n-propyl- $\omega$ -sulfonic acids.

According to the dual substituents R and X, the primary addition agents of the invention are of four general types in each of which the nature of the substituent R' is not particularly critical as long as it does not reduce the solubility of the compound below the lower limit of effectiveness.

The compounds of the first type in which X is oxygen and R is hydrogen are preferably employed in concentrations between 0.5 millimole per liter and their upper limit of solubility or approximately five millimoles per liter, whichever is lower. No further desirable changes in deposit properties are achieved by exceeding the concentration of five millimoles per liter where solubility is adequate.

The following compounds are representative of the first type of primary addition agent:

- (1) N-(tetrahydropyran-2)-acetamide
- (2) N-(tetrahydropyran-2)-propionamide
- (3) N-(tetrahydropyran-2)-butyramide
- (4) N-(tetrahydropyran-2)-benzamide
- (5) N-(tetrahydropyran-2)-p-toluaamide
- (6) N-(tetrahydropyran-2)-nicotinamide
- (7) N-(tetrahydropyran-2)-picolinamide
- (8) N-(tetrahydropyran-2)N'-acetylurea
- (9) N-(tetrahydropyran-2)-N'-carbethoxyurea
- (10) N-(tetrahydropyran-2)-N'-phenylsulfonylurea
- (11) N-(tetrahydropyran-2)-N'-nitrourea
- (12) N-(tetrahydropyran-2)-N'-carboxyurea

The second type of primary addition agent differs from the first type by the substitution of a radical



for the hydrogen atom in position R of the compounds of the first type. All compounds of the first type enumerated above for the sake of illustration may be converted to the second type by reaction with propane sultone. The twelve compounds so obtained are readily soluble, and their brightening effects increase over a wider range of concentrations than those of the first type of primary brighteners. The second type of primary addition agents is preferably employed at concentrations of 0.5 millimole per liter and higher, and their favorable effects increase up to a concentration of 0.01 mole per liter.

The third type of primary addition agents according to the invention differs from the first type by substitution of sulfur for the oxygen in position X. The thiamides of the third type are more effective than the corresponding substituted amides of the first type at equal concentrations, and are preferably employed over a range of 0.2 millimole to five millimoles per liter or to their limit of

solubility whichever is lower. The following compounds are representative of the third type:

- (13) N-(tetrahydropyran-2)-thioacetamide
- (14) N-(tetrahydropyran-2)-thiopropionamide
- (15) N-(tetrahydropyran-2)-thiobutyramide
- (16) N-(tetrahydropyran-2)-thiobenzamide
- (17) N-(tetrahydropyran-2)-p-thiotoluamide
- (18) N-(tetrahydropyran-2)-thiourea
- (19) N-(tetrahydropyran-2)-N'-acetylthiourea
- (20) N-(tetrahydropyran-2)-N'-carbethoxythiourea
- (21) N-(tetrahydropyran-2)-N'-formylthiourea
- (22) N-(tetrahydropyran-2)-N'-cyanothiourea
- (23) N-(tetrahydropyran-2)-N'-carboxythiourea
- (24) N-(tetrahydropyran-2)-N'-phenylsulfonylthiourea
- (25) N-(tetrahydropyran-2)-N'-nitrothiourea
- (26) N-(tetrahydropyran-2)-N'-allylthiourea
- (27) N-(tetrahydropyran-2)-N'-phenylthiourea

The fourth type of primary addition agent of the invention differs from the second type by the presence of sulfur in position X of the formula, and representative compounds of the fourth type are obtained by reaction of propane sultone with each of the compounds (13) to (27) enumerated hereinabove. The compounds of the fourth type are employed over the same range of concentrations as those of the second type.

The primary brightening agents of the invention are highly effective in both types of acid copper plating solutions presently in commercial use, namely the sulfate type and the fluoborate type. Their use with electroplating solutions of these types is illustrated by the following examples, but it will be understood that the invention is not limited to the examples.

#### Example 1

A copper plating solution was prepared from

|                                                           |        |
|-----------------------------------------------------------|--------|
| Copper sulfate, cryst., grams per liter -----             | 200    |
| Sulfuric acid, C.P., grams per liter -----                | 50     |
| N-(tetrahydropyran-2)-nicotinamide, moles per liter ----- | 0.0009 |

Copper was deposited from the solution under the following conditions:

|                                                                |          |
|----------------------------------------------------------------|----------|
| Temperature, ° C. -----                                        | 22 to 26 |
| Cathode current density, amps. per square foot (average) ----- | 45       |
| Agitation (cathode movement), meters per min. -----            | 2 to 8   |

Fully bright deposits were formed on all surfaces on which the actual current density was between 4.5 and 72 amps. per square foot. Depressions in the base metal (brass) of 40 microns depth were practically completely obliterated when the average thickness of the deposit reached 20 microns.

These results are typical of the brightening compounds of the first type, and were substantially duplicated with each of the compounds enumerated above sub (1) to (12) in equimolecular amounts.

#### Example 2

A copper plating electrolyte was prepared from

|                                                            |        |
|------------------------------------------------------------|--------|
| Copper fluoborate, grams per liter -----                   | 250    |
| Fluoboric acid, grams per liter -----                      | 30     |
| N-(tetrahydropyran-2)-N'-acetylurea, moles per liter ----- | 0.0012 |

The following operating conditions were maintained during plating:

|                                                              |          |
|--------------------------------------------------------------|----------|
| Temperature, ° C. -----                                      | 22 to 28 |
| Cathode current density, amps. per square foot average ----- | 54       |
| Agitation (cathode movement), meters per min. -----          | 2 to 8   |

The deposits formed were fully bright over an actual cathode current density range of 6.3 to 81 amps. per

square foot as determined on a bent brass sheet electrode, and had a good leveling effect.

Closely similar effects were achieved with the other compounds of the first type enumerated above sub (1) to (12).

#### Example 3

The composition and operating conditions of a copper plating solution were as follows:

|                                                                                               |          |
|-----------------------------------------------------------------------------------------------|----------|
| 10 Copper sulfate, cryst., grams per liter -----                                              | 200      |
| Sulfuric acid, C.P., grams per liter -----                                                    | 60       |
| N-(tetrahydropyran-2)-N-(n-propane- $\omega$ -sulfonic acid)-acetamide, moles per liter ----- | 0.003    |
| 15 Temperature, ° C. -----                                                                    | 20 to 28 |
| Cathode current density, amps. per sq. ft. -----                                              | 45       |
| Agitation (cathode movement), meters per min. -----                                           | 2 to 8   |

The coating produced were bright, pore-free, and of very high ductility. Scratches in the base metal having a depth of 40 microns were practically completely leveled when the average thickness of the copper coating reached 20 microns.

Closely similar results were obtained under otherwise comparable conditions when the brightening agent used was replaced by the other products of the reaction between propane sultone and the compounds of the first type listed sub (1) to (12).

#### Example 4

A copper plating solution of the composition listed below was used under the indicated operating conditions:

|                                                                                                       |          |
|-------------------------------------------------------------------------------------------------------|----------|
| 35 Copper fluoborate, grams per liter -----                                                           | 300      |
| Fluoboric acid, grams per liter -----                                                                 | 40       |
| N-(tetrahydropyran-2)-N-(n-propane- $\omega$ -sulfonic acid)-N'-carbethoxyurea, moles per liter ----- | 0.004    |
| 40 Temperature, ° C. -----                                                                            | 20 to 28 |
| Cathode current density, amps. per sq. ft. -----                                                      | 63       |
| Agitation (cathode movement), meters per min. -----                                                   | 2 to 8   |

The copper coatings produced were fully bright over an actual cathode current density range of 5.4 to 90 amps. per square foot as determined with a bent brass sheet cathode, and had a very good leveling effect. Closely similar results were obtained with the other brightening compounds referred to in Example 3.

#### Example 5

Mirror bright copper deposits free from pores and of very good ductility were produced from an electrolyte of the following composition under the operating conditions listed:

|                                                              |          |
|--------------------------------------------------------------|----------|
| 60 Copper sulfate, cryst., grams per liter -----             | 200      |
| Sulfuric acid, C.P., grams per liter -----                   | 60       |
| N-(tetrahydropyran-2)-p-thiotoluamide, moles per liter ----- | 0.0006   |
| 65 Temperature, ° C. -----                                   | 22 to 26 |
| Cathode current density, amps per sq. ft. average -----      | 45       |
| Agitation (cathode movement), meters per min. -----          | 2 to 8   |

The copper plate was fully bright over an actual cathode current density range from 2.7 to 72 amps. per square foot. Scratches in the base metal having a depth of 40 microns were practically leveled when the average coating thickness reached 15 microns. Equimolecular amounts of the other compounds of the third type listed above under numbers (13) to (27) gave corresponding results.

## Example 6

Mirror bright copper deposits were obtained from a fluoborate electrolyte having the following composition, and operated under the listed conditions:

|                                                           |          |
|-----------------------------------------------------------|----------|
| Copper fluoborate, grams per liter                        | 250      |
| Fluoboric acid, grams per liter                           | 40       |
| N-(tetrahydropyran-2)-N'-carboxythiourea, moles per liter | 0.001    |
| Temperature, °C.                                          | 20 to 26 |
| Cathode current density, amps. per sq. ft. average        | 54       |
| Agitation (cathode movement), meters per min.             | 2 to 8   |

The deposits were formed on objects of complex configuration, yet they were fully bright when their thickness reached 2 microns, and were still brilliantly and uniformly bright at an average deposit thickness of 200 microns. The leveling effect was good, and the copper plate did not show pores although no addition agent other than that of the invention had been employed.

Corresponding results were obtained with equimolecular amounts of the other compounds of the third type listed hereinabove.

## Example 7

A sulfate type copper plating bath was prepared and operated as follows:

|                                                                                                 |          |
|-------------------------------------------------------------------------------------------------|----------|
| Copper sulfate, cryst., grams per liter                                                         | 200      |
| Sulfuric acid, C.P., grams per liter                                                            | 60       |
| N-(tetrahydropyran-2)-N-(n-propane- $\omega$ -sulfonic acid)-N'-acetylthiourea, moles per liter | 0.0015   |
| Temperature, °C.                                                                                | 20 to 28 |
| Cathode current density, amps. per sq. ft.                                                      | 45       |
| Agitation (cathode movement), meters per min.                                                   | 2 to 8   |

The coatings produced were mirror bright from 1.8 to 72 amps. per square foot of actual cathode current density. They were ductile and free from visible pores. Irregularities in the base metal having a depth of 40 microns were completely leveled when the average thickness of the deposit reached 15 microns.

Similarly favorable results were obtained with the other reaction products of propane sulfone with the compounds of the third type listed sub (13) to (27). Peak performance was obtained from the several compounds at concentrations varying between 0.001 and 0.003 mole per liter.

## Example 8

Very ductile copper electrodeposits having good leveling action and being mirror bright were obtained from a fluoborate bath as follows:

|                                                                                                 |          |
|-------------------------------------------------------------------------------------------------|----------|
| Copper fluoborate, grams per liter                                                              | 250      |
| Fluoboric acid, grams per liter                                                                 | 30       |
| N-(tetrahydropyran-2)-N-(n-propane- $\omega$ -sulfonic acid)-N'-allyl thiourea, moles per liter | 0.0024   |
| Temperature, °C.                                                                                | 20 to 28 |
| Cathode current density, amps per sq. ft. average                                               | 54       |
| Agitation (cathode movement), meters per min.                                                   | 2 to 8   |

Full brightness was achieved over an actual cathode current density range from 3.6 to 81 amps. per square foot.

The other compounds of the fourth type gave similar brilliantly bright copper deposits when employed as brighteners in the fluoborate electrolyte under the indicated operating conditions.

The secondary addition agents of the invention enhance the desirable properties of copper plating solutions containing the primary agents by increasing the range of current densities at which mirror bright or fully bright de-

posits can be obtained, particularly at operating temperatures of 25 to 50° C., and by further improving the leveling effects of the bath.

The secondary addition agents are amines of the formula



or corresponding ammonium salts of the formula



wherein  $R_1$  is tetrahydropyranyl (I) or tetrahydrofuryl (II)

(I)



(II)



$R_2$  and  $R_3$  are hydrogen, lower alkyl, phenyl, 2-carboxyphenyl, 4-hydroxyphenyl, 4-sulfophenyl, p-diphenyl, 2-pyridyl, 6,8-disulfo-2-naphthyl, the sulfo radical  $-SO_3H$ , or a radical  $-(CH_2)_n-SO_3H$  wherein  $n$  is an integer not greater than 4, and preferably 3 or 4, and  $R_4$  is lower alkyl. When  $R_2$  is different from lower alkyl,  $R_3$  is a member of the last mentioned group different from  $R_2$ .  $A^-$  may be the anion of any organic or inorganic acid. The nature of the anion is generally irrelevant since the desirable effects of the ammonium salts are due entirely to the cationic component.

The following compounds are representative of the secondary addition agents of the invention:

- (1) N-2-tetrahydropyranyl-N-methylamine
- (2) N-2-tetrahydropyranyl-N-2-carboxyphenylamine
- (3) N-2-tetrahydropyranyl-N-2-carboxyphenyl-N-methylamine
- (4) N-2-tetrahydropyranyl-N-4-hydroxyphenylamine
- (5) N-2-tetrahydropyranyl-N- $\omega$ -sulfo-n-butylamine
- (6) N-2-tetrahydropyranyl-N- $\omega$ -sulfo-n-propylamine
- (7) N-2-tetrahydropyranyl-aniline
- (8) N-2-tetrahydropyranyl-N-2-pyridyl-N- $\omega$ -sulfo-n-propylamine
- (9) N-2-tetrahydropyranyl-N-6,8-disulfo-2-naphthyl-N- $\omega$ -sulfo-n-propylamine
- (10) N-2-tetrahydropyranyl-N-2-carboxyphenyl-N- $\omega$ -sulfo-n-butylamine
- (11) N-2-tetrahydropyranyl-N-trimethylammonium sulfate
- (12) N-2-tetrahydropyranyl-N-4-hydroxyphenyl-N-dimethylammonium chloride
- (13) N-2-tetrahydrofuryl-N-methylamine
- (14) N-2-tetrahydrofuryl-N-4-sulfophenyl-N- $\omega$ -sulfo-n-propylamine
- (15) N-2-tetrahydrofuryl-N-2-pyridyl-N- $\omega$ -sulfo-n-butylamine
- (16) N-2-tetrahydrofuryl-N-4-hydroxyphenyl-N-dimethylammonium chloride
- (17) N-2-tetrahydropyranyl-N-p-diphenyl-1-amine
- (18) N-2-tetrahydropyranyl-N-sulfo-amine

The secondary addition agents of the invention may be added to the copper plating solutions described in Examples 1 and 8 in amounts of 0.05 to 2.0 grams per liter. The effects produced vary with concentration in the same manner as described hereinabove with reference to the primary brightening or addition agents. The range of permissible operating conditions is increased by the secondary

agents, brightness and brightness range are improved, particularly at higher temperatures.

All secondary addition agents of the invention are beneficial to the several types of plating solutions enumerated in the examples, and may be combined with all the primary addition agents specifically described hereinabove. The following example is merely typical of the results obtained.

*Example 9*

A sulfate type copper plating bath was prepared as described in Example 7, but the solution additionally contained as a secondary addition agent 0.003 mole per liter of N-2-tetrahydropyranyl - N-2-pyridyl-N- $\omega$ -sulfo- $\omega$ -propylamine. Without loss of brightness, the bath could be operated at an average current density of 90 amps. per square foot, and the temperature could be permitted to rise to 50° C. Ductility and freedom from pores were not impaired, and leveling was improved as indicated by disappearance of irregularities in the base metal at an average thickness lower than that of Example 7.

It will be appreciated that the acid copper sulfate and copper fluoborate electrolytes described in Examples 1 to 9 are entirely conventional in composition except for the brightening agents of the invention, and that the operating conditions employed are not unusual. The effects of the constituents in these solutions are well known, and those skilled in the art will find that variations in the concentrations of copper salts and free acids in these electrolytes affect the bright deposits of the invention in a manner analogous to the effects produced in the absence of the brightening agents.

The temperature of the solutions is not critical. No effort was made in the plating runs reported on in the examples to hold the temperature within specific limits. The brightening agents of the invention are effective at temperatures as low as 10° C. or as high as 50° C. It is not usually necessary to employ copper sulfate or copper fluoborate plating solutions outside these extreme temperatures. An operating temperature between 10° C. and 50° C. is readily maintained without heating or cooling of the electrolyte under the ambient conditions of temperature prevailing in almost any plating plant.

The coatings produced do not lose their brightness or smoothness as their thickness increases. Coatings having a thickness of one millimeter (0.04 inch) are still fully bright, ductile, and dense.

The addition agents of the invention are chemically stable in acid copper electrolytes when obviously unstable substituents are avoided. They are consumed at a low rate during current passage through the electrolyte, and this rate is readily determined for a given plating installation so that replenishment of brightening agents may be based on measurements of ampere hours of current passed.

Bright deposits can be obtained with the brightening agents of the invention up to cathode current densities of about 90 amps. per square foot without agitation. Current densities much higher than 90 amps. per square foot are entirely practical with suitably rapid relative movement of electrolyte and plated object.

The brightening agents of the invention are relatively insensitive against contaminating ions such as those of lead, zinc, nickel, divalent and trivalent iron, and even hexavalent chromium. Copper plating solutions of the invention thus produce electrodeposits of the desired properties when made up of commercial chemicals of the grades normally employed in the electroplating industry without requiring purification by chemical treatments, electrolysis at low current density, or the like.

While the invention has been described with particular reference to specific embodiments, it is to be understood that it is not limited thereto, but is to be construed broadly and restricted solely by the scope of the appended claims.

What is claimed is:

1. An aqueous acid copper plating electrolyte contain-

ing as a primary brightening agent an effective amount of an N-(tetrahydropyranyl-2) amide of a carboxylic acid dissolved in said electrolyte; and as a secondary brightening agent an effective amount of an amine of the formula



10 or an ammonium ion of the formula



15 in said formulas R<sub>1</sub> being tetrahydropyranyl or tetrahydronfuryl; R<sub>2</sub> and R<sub>3</sub> being hydrogen, lower alkyl, phenyl, 2-carboxyphenyl, 4-hydroxyphenyl, 4-sulfophenyl, p-phenyl, 2-pyridyl, 6,8-disulfo-2-naphthyl, or a sulfonic acid radical  $-(CH_2)_n-SO_3H$  wherein n is an integer not greater than 4; said R<sub>3</sub> being different from R<sub>2</sub> when said R<sub>2</sub> is different from lower alkyl; and R<sub>4</sub> being lower alkyl.

20 2. An aqueous acid copper plating electrolyte containing as a primary brightening agent an effective amount of an N-(tetrahydropyranyl-2) amide of a thiocarboxylic acid dissolved in said electrolyte; and as a secondary brightening agent an effective amount of an amine of the formula



30 or an ammonium ion of the formula



35 40 in said formulas R<sub>1</sub> being tetrahydropyranyl or tetrahydronfuryl; R<sub>2</sub> and R<sub>3</sub> being hydrogen, lower alkyl, phenyl, 2-carboxyphenyl, 4-hydroxyphenyl, 4-sulfophenyl, p-phenyl, 2-pyridyl, 6,8-disulfo-2-naphthyl, or a sulfonic acid radical  $-(CH_2)_n-SO_3H$  wherein n is an integer not greater than 4; said R<sub>3</sub> being different from said R<sub>2</sub> when said R<sub>2</sub> is different from lower alkyl; and R<sub>4</sub> being lower alkyl.

45 50 5. An aqueous acid copper plating electrolyte containing as a primary brightening agent an effective amount of an N-(tetrahydropyranyl-2)-N-(propane- $\omega$ -sulfonic acid) amide of a carboxylic acid dissolved in said electrolyte; and as a secondary brightening agent an effective amount of an amine of the formula



55 or an ammonium ion of the formula



60 65 in said formulas R<sub>1</sub> being tetrahydropyranyl or tetrahydronfuryl; R<sub>2</sub> and R<sub>3</sub> being hydrogen, lower alkyl, phenyl, 2-carboxyphenyl, 4-hydroxyphenyl, 4-sulfophenyl, p-phenyl, 2-pyridyl, 6,8-disulfo-2-naphthyl, or a sulfonic acid radical  $-(CH_2)_n-SO_3H$  wherein n is an integer not greater than 4; said R<sub>3</sub> being different from said R<sub>2</sub> when said R<sub>2</sub> is different from lower alkyl; and R<sub>4</sub> being lower alkyl.

70 75 7. An aqueous acid copper plating electrolyte containing as a primary brightening agent an effective amount of an N-(tetrahydropyranyl-2) - N-propane- $\omega$ -sulfonic acid amide of a thiocarboxylic acid dissolved in said elec-

troyte; and as a secondary brightening agent an effective amount of an amine of the formula



or an ammonium ion of the formula



in said formulas  $R_1$  being tetrahydropyranyl or tetrahydrofuryl;  $R_2$  and  $R_3$  being hydrogen, lower alkyl, phenyl, 2-carboxyphenyl, 4-hydroxyphenyl, 4-sulfophenyl, p-diphenyl, 2-pyridyl, 6,8-disulfo-2-naphthyl, or a sulfonic acid radical  $-(CH_2)_n-SO_3H$  wherein  $n$  is an integer not greater than 4; said  $R_3$  being different from said  $R_2$  when said  $R_2$  is different from lower alkyl; and  $R_4$  being lower alkyl.

5. An aqueous acid copper plating electrolyte comprising copper sulfate or copper fluoborate as a source of copper ions, sulfuric acid or fluoboric acid as a source of hydrogen ions, an effective amount of a primary brightening agent of the formula



wherein  $X$  is oxygen or sulfur,  $R$  is hydrogen or the radical  $-CH_2-CH_2-SO_3H$ , and  $R'$  is lower alkyl, phenyl, pyridyl, or a radical of the formula  $-NHR''$ , wherein  $R''$  is hydrogen, lower alkenyl, lower alkanoyl, carboxy, carbo-(lower)-alkoxy, phenylsulfonyl, nitro, formyl, cyano, or phenyl; and as a secondary brightening agent an effective amount of an amine of the formula



or an ammonium ion of the formula



in said formulas  $R_1$  being tetrahydropyranyl or, tetrahydrofuryl;  $R_2$  and  $R_3$  being hydrogen, lower alkyl, phenyl, 2-carboxyphenyl, 4-hydroxyphenyl, 4-sulfophenyl, p-diphenyl, 2-pyridyl, 6,8-disulfo-2-naphthyl, or a sulfonic

50

45

25

30

35

40

45

acid radical  $-(CH_2)_n-SO_3H$  wherein  $n$  is an integer not greater than 4; said  $R_3$  being different from said  $R_2$  when said  $R_2$  is different from lower alkyl; and  $R_4$  being lower alkyl.

6. A method of producing a bright, smooth, pore-free, and ductile copper coating on a conductive object which comprises making said object a cathode in an aqueous electrolyte containing copper sulfate or copper fluoborate as a source of copper ions, sulfuric acid or fluoboric acid as a source of hydrogen ions, a primary brightening agent, and a secondary brightening agent, said sources and said agents being dissolved in said solution, said primary agent being a  $N$ -(tetrahydropyranyl-2) amide of a carboxylic or thiocarboxylic acid, or an  $N$ -(tetrahydropyranyl-2)- $N$ -(propane- $\omega$ -sulfonic acid) amide of a carboxylic or thiocarboxylic acid, said secondary brightening agent being an amine of the formula



or an ammonium ion of the formula



in said formulas  $R_1$  being tetrahydropyranyl or tetrahydrofuryl;  $R_2$  and  $R_3$  being hydrogen, lower alkyl, phenyl, 2-carboxyphenyl, 4-hydroxyphenyl, 4-sulfophenyl, p-diphenyl, 2-pyridyl, 6,8-disulfo-2-naphthyl, or a sulfonic acid radical  $-(CH_2)_n-SO_3H$  wherein  $n$  is an integer not greater than 4; said  $R_3$  being different from said  $R_2$  when said  $R_2$  is different from lower alkyl; and  $R_4$  being lower alkyl, the concentration of said primary brightening agent in said electrolyte being between 0.2 and ten millimoles per liter, the concentration of said secondary brightening agent in said electrolyte being between 0.05 and 2.0 grams per liter, and the temperature of said electrolyte being between 10° C. and 50° C.

#### References Cited

##### UNITED STATES PATENTS

2,837,472 6/1958 Gundel et al. 204-52 X

##### FOREIGN PATENTS

1,168,207 4/1964 Germany.

JOHN H. MACK, Primary Examiner.

G. KAPLAN, Assistant Examiner.